

# UNITED STATES PATENT OFFICE.

LAURENCE H. WHITNEY, OF PITTSFIELD, MASSACHUSETTS, ASSIGNOR TO GENERAL ELECTRIC COMPANY, A CORPORATION OF NEW YORK.

## PROCESS OF ANNEALING ALUMINUM.

1,273,706.

Specification of Letters Patent. Patented July 23, 1918.

No Drawing.

Application filed May 7, 1917. Serial No. 166,823.

To all whom it may concern:

Be it known that I, LAURENCE H. WHITNEY, a citizen of the United States, residing at Pittsfield, in the county of Berkshire, 5 State of Massachusetts, have invented certain new and useful Improvements in Processes of Annealing Aluminum, of which the following is a specification.

The present invention relates to the annealing of aluminum after the metal has been rendered hard by mechanical working, and the object of my invention is to produce aluminum articles in which the unavoidable silicon impurity is substantially all in the 15 dissolved state instead of being present as graphitoidal silicon. The product of my invention is of particular utility in electrolytic cells, such as lightning arresters, but in its use is not necessarily limited to such 20 devices.

Aluminum unavoidably contains about 0.20% of silicon. When aluminum is fused and cast the greater part of the silicon is found to be present in the dissolved state. 25 Upon mechanical working of the cast metal into desired shape, it is hardened so as to require annealing. I have found that by annealing the metal as heretofore practised, a large percentage of the previously dissolved silicon is converted into the graphitoidal state. The graphitoidal silicon in the aluminum is deleterious to the formation of a film on the aluminum when used as electrode material for electrolytic cells, such 35 as, for example, lightning arresters. Chemically, this conversion is distinguishable by the dark color of the residue from dehydrating the dissolved sample in certain mineral acids. This residue contains the graphitic 40 or metallic silicon and silicon dioxid. From this residue the metallic silicon can be determined by a well-known electrochemical method.

In accordance with my invention, I have 45 produced annealed aluminum by subjecting the metal to a temperature intermediate between about 370° C. and 450° C. until softened, and cooling rapidly. If the aluminum sheets are heated to a temperature substantially 50 in excess of 450° C. the metal is rendered unfit for use in electrolytic cells. The first effect upon the metal as this temperature is exceeded is the formation of numerous protuberances looking like small blisters 55 or warts upon the metal surface as though

gas bubbles were forming in the metal. Metal subjected to temperatures much higher than 450° C. is darkened in color and has a peculiar glazed or varnished appearance, while the protuberances are larger and 60 more numerous. My invention also includes the new product resulting from the practice of my invention.

In carrying out my invention, the metal is cast as usual into any shape suitable for 65 subsequent mechanical treatment, such as drawing, spinning, stamping, forging or the like. During the desired mechanical treatment which is carried out as usual, the metal unavoidably becomes hardened. Thereupon 70 the shaped or worked articles are placed in a furnace which may be heated and cooled quickly, for example, an electric muffle furnace, and heated rapidly to a temperature in excess of 370° C., and preferably below 75 450° C. The annealing treatment is continued for about 2½ to 3 hours. The aluminum articles then are removed from the furnace and are quickly cooled, for example, if the articles are large, by blowing air 80 upon them or by quenching them in water. Smaller articles may be sufficiently rapidly cooled by merely exposing to the air.

The formation of graphitic silicon appears to be dependent both on the temperature and on the length of time the metal is subjected to the temperature at which graphitic silicon is formed. Apparently there is a critical temperature below 370° C. at 85 which the transformation of dissolved silicon into graphitic silicon takes place rapidly. Therefore, it is important in the cooling down of the softened metal, not to allow it to remain any longer than necessary at the temperatures below 370° where conversion takes place. 90

What I claim as new and desire to secure by Letters Patent of the United States, is:—

1. The process of annealing aluminum rendered hard by mechanical working and 100 containing dissolved silicon which consists in subjecting the metal until softened to a heat treatment above the temperature at which dissolved silicon is converted into graphitic silicon, but below the temperature 105 at which the metal surface becomes uneven and darkened, and then cooling the aluminum so rapidly to ordinary temperature that the formation of appreciable graphitoidal silicon is avoided. 110

2. The process of annealing aluminum containing dissolved silicon and which has been rendered hard by mechanical working, which consists in rapidly carrying the metal  
5 to a temperature within the range of about 370° C. and 450° C., maintaining a temperature within said range until the aluminum

is softened and then quickly chilling the metal, thereby preventing the formation of appreciable graphitoidal silicon at tempera- 10  
tures below said range.

In witness whereof, I have hereunto set  
my hand this third day of May 1917.

LAURENCE H. WHITNEY.